# EUROPEAN PATENT SPECIFICATION

(11) **EP 2 138 250 B1**
(45) Date of publication and mention of the grant of the patent: **24.12.2014**
(21) Application number: 09163363.6
(22) Date of filing: 22.06.2009
(51) Int. Cl.: B21D 53/30

(54) **Method for manufacturing discs for wheels, particularly for commercial vehicles**
Herstellungsverfahren für Radscheiben, insbesondere für Nutzfahrzeuge
Procédé de fabrication de disques pour roues, particulièrement pour des véhicules commerciaux

(30) Priority: 23.06.2008 IT TO20080491
(43) Date of publication of application: 30.12.2009
(73) Proprietor: GIANETTI RUOTE S.R.L., 20816 Ceriano Laghetto (MB) (IT)
(72) Inventor: Finzi, Andrea, I-20050, Tregasio Frazione di Triuggio (Milano) (IT); Bazzoni, Davide, I-21040, Cislago (Varese) (IT); Perris Magnetto, Gabriele, I-10098, Rivoli (Torino) (IT)
(74) Representative: Quinterno, Giuseppe

(56) References cited:
- EP-A1- 1 867 408
- JP-A- 2005 000 967
- JP-A- 2005 007 407
- US-A- 1 931 163
- US-A- 2 983 033

## Description

The present invention refers to wheels for motor vehicles of the type comprising a rim to which a disc is welded, and concerns in particular a method for manufacturing a disc, of the kind defined in the preamble of claim 1.

Such a type of method is described in EP-1867408-A.

The method described in said document provides that the starting strip of sheet metal is bent on its entire extension, and its end portions, correspondingly arched, are brought together and butt welded. The butt welding of such end portions to obtain a cylindrical ring is indeed problematic. The thus obtained cylindrical ring is then directly subjected to a first press-moulding operation, to shape it into a truncated-cone or annular sphere segment. Also this radical change of shape is problematic.

JP-2005 000 967 A discloses a method for manufacturing a rim of a wheel, starting from a planar, rectangular strip of an aluminium alloy. Said strip is rounded and the ends thereof are flattened and joined by a friction stir welding apparatus which also makes said ends thinner.

US 1 931 163 A discloses a method of making a hub shell for a wire wheel starting from a rectangular strip of metal. The strip is rounded and its ends are flattened and joined by upset welding. Following the removal of weld flashes and burrs, the thus obtained cylindrical ring is directly subjected to pressing and shaping operations to bring it to a desired final shape.

One purpose of the present invention is therefore that of putting forward an improved method of the type specified above.

These and other purposes are obtained according to the invention with a method having the features defined in claim 1.

Further characteristics and advantages of the invention shall become clear in the following detailed description, given simply as an example with reference to the attached drawings, in which:
figure 1 is a plan view of a sheet of sheet metal used for making a wheel disc according to the invention;
figure 2 is a perspective view of a ring obtained by bending and welding the end portions, left on the same plane, of the sheet of sheet metal of figure 1;
figure 3 is a partial side view of the ring shown in figure 2;
figure 4 is a perspective view of a ring obtained starting from that in figure 2, through an operation of rounding by radial expansion carried out on an axial portion of such a ring;
figure 5 is a perspective view of an annular shell element obtainable starting from the ring of figure 4 through a pressing operation;
figures 6 and 7 are perspective views, partially sectioned, which show the tools for two successive pressing operations;
figure 8 is a perspective view of an annular shell element obtained through operations of flow forming: and
figure 9 is a perspective view of a wheel disc obtained starting from the shell element of figure 8, through final shearing operations of openings or windows.

With reference to the drawings, in the method according to the invention the making of a disc of a wheel for a motor vehicle begins with the provision of a strip of sheet metal, indicated with 1 in figure 1, having a general shape like an elongated parallelogram, preferably with a rectangular shape, and having an essentially uniform thickness.

In the case of a wheel for a truck or other commercial/industrial vehicles, such a thickness can be, for example, about 8-16 mm.

The strip of sheet metal 1 is then shaped: it is mainly bent, leaving however, that its end portions or limbs, indicated with 1a and 1b in figures 1 and 2, remain level. The end faces of the limbs 1a and 1b of the strip 1 are brought together, and then welded, on substantially a same plane, so as to make a substantially cylindrical ring 2, which has a chordal flattened wall portion, formed by the two limbs 1a and 1b brought together and welded.

With reference to figure 3, the central axis of the ring 2 is indicated O, and the flattened limbs 1a and 1b are advantageously subtended by an angle α having extension between 5° and 15°, and preferably equal to about 10°.

The bringing together, and then the butt welding, of the end limbs 1a and 1b is extremely easy, and does not require special tools. In fact, bringing together said limbs on substantially a same plane improves the matching of the end surfaces or faces of said limbs, making it uniform. The subsequent excess metal removal processes at the welding are also easier, as are the subsequent finishing operations of the welded area.

The mechanical characteristics of the welds thus made have a narrower variation range, with a substantial improvement of the general quality.

After the welding and the following accessory processes, but before the subsequent pressing and shaping operations, the ring 2 of figure 2 is subjected to a preliminary rounding operation through radial expansion with *per se* known tools.

In such a rounding operation the expansion is of greater magnitude in a first axial portion of the ring 2, so that the remaining axial portion of such a ring takes a substantially cone-shaped configuration. Figure 4 shows the ring 2 after such an operation: the lower portion 2a subjected to radial expansion is substantially cylindrical, whereas the remaining axial portion 2b is essentially shaped like a truncated cone. The height hₐ of the expanded portion 2a is preferably greater than that of the remaining portion 2b. Advantageously, the height hₐ can be equal to about three times the height h_{b}.

The extent to which the portion 2b is shaped like a cone, expressed as the difference in radius Δr between its ends (figure 4), can take values of about 1-5 mm.

After the aforementioned preliminary rounding operation, the ring 2 is advantageously subjected to a material removal process, in particular turning, to bring the axial height or length to a predetermined nominal value, and to make its circular end edges level and parallel with each other. Such an operation is extremely important, as it allows possible imperfections of alignment and welding of the two end limbs 1a and 1b of the initial strip 1 to be eliminated, avoiding that in the following operations of plastic deformation of the ring, it suffers anomalous stress and reducing the effects of wear due to press-moulding tools.

In the aforementioned material removal process advantageously the corners of the edges of the ring 2 which must drag against the moulds or shapes in the following operations are bevelled or rounded.

The ring 2 is then subjected to press-moulding operations.

In a first moulding operation the edge with the greatest diameter of the ring 2 is axially brought into abutment against a stop surface, so that the material of the ring is made to flow radially towards the centre, at its edge with smaller diameter.

Figure 5 of the attached drawings shows an annular shell element 3 obtained through such a first moulding operation, made for example with (*per se* known) tools schematically and partially illustrated in figure 6. Such tools comprise an upper mould 10 and a lower matching mould 11, where the latter has an annular abutment or stop surface 11a for the edge of the ring with greater diameter.

By comparing figures 4 and 5 it can be quickly gathered how through the first moulding operation, the annular shell 3 has a smaller diameter that is smaller than the corresponding diameter of the starting ring 2, and a larger diameter that is substantially larger than the corresponding diameter of the starting ring. Moreover, the axial height or length of the annular shell 3 is shorter than the height of the starting ring 2.

The first moulding operation is advantageously followed by a second one, in which the material of the ring is made to flow radially towards the centre, at its edge with the smaller diameter, whereas the material at its edge with greater diameter is made to flow radially outwards and longitudinally. This can be made, for example, with the tools schematically and partially illustrated in figure 7, in which the upper mould 13, in addition to what has already been described, has, at the bottom, a central cylindrical ridge 13a, functioning as a "centrer" intended to define the diameter of the smallest opening 4a of the annular shell obtained through said second moulding operation (as seen in particular in figure 8).

The semi-finished element 4 can then be subjected to forming operation with a lathe to reach the intended distribution of thickness, and of shearing, for making in such a semi-finished element a plurality of openings or windows, intended for example to allow fixing elements of the disc-wheel to pass to the corresponding wheel hub, as ventilation openings, or simply for aesthetic purposes as shown, for example, in figure 9.

Advantageously, the starting strip of sheet metal 1 (figure 1) is made in steel, in particular steel with low alloying element content, for example steel having a manganese content substantially between 0.15% and 0.80% of the total weight, and having a stretching percentage greater than 25%.

Of course, the principle of the invention remaining the same, the embodiments and the details can be widely varied with respect to what has been described and illustrated purely as an example , without for this reason departing from the scope of the invention as defined in the attached claims.

## Claims

1. Method for manufacturing a disc (4) for a wheel of a motor vehicle, comprising the operations of:
- providing a strip of sheet metal (1) substantially shaped like an elongated parallelogram with an essentially uniform thickness;
- bending said strip of sheet metal (1) and welding together the end portions (1a, 1b) thereof so as to form a substantially cylindrical ring; and
- subjecting said ring (2) to pressing and shaping operations through plastic deformation so as to give it a desired shape;
the method being **characterized in that**:
- the strip of sheet metal (1) is bent so that its end portions (1a, 1b) are level;
- said end portions (1a, 1b) are brought together and butt welded substantially on a same plane, so as to obtain a ring (2) which has a chordal flattened wall portion (1a, 1b);
- before undergoing the aforementioned pressing and shaping operations, said ring (2) is subjected to a preliminary rounding operation,
and **in that**
- said rounding operation is performed through radial expansion such that the expansion is of a greater magnitude in a first, substantially cylindrical, axial portion (2a) of the ring (2), and the remaining axial portion (2b) of the ring (2) takes a substantially cone-shaped configuration.

2. Method according to claim 1, wherein the aforementioned remaining axial portion (2b) of the ring (2) which has a substantially cone-shaped configuration, extends over about 25% of the axial height or length of the ring (2).

3. Method according to claim 1 or 2, wherein, after the aforementioned preliminary rounding operation and before said pressing and shaping operations, said ring (2) is subjected to an operation of material removal, in particular a turning operation, to bring its height or axial length to a predetermined nominal value, and to make its end edges level and parallel to each other.

4. Method according to claim 3, wherein, in said operation of material removal, the corners of the edges of the ring (2) which must drag against the moulds or shapes in the following operations are bevelled or rounded.

5. Method according to any one of the previous claims, wherein the aforementioned level end portions (1a, 1b) have an extension such that in cross-section they are each subtended by an angle (α) between 5° and 15°, and preferably of around 10°, said angle (α) having vertex on the axis (0) of the ring (2).

6. Method according to any one of the previous claims, wherein said pressing operations comprise a first moulding operation which is carried out after said preliminary rounding operation, and in which the edge with the greatest diameter of the ring (2) is axially brought into abutment against a stop surface (11a), so that the material of the ring (2) is then made to flow radially towards the centre, at the edge with smaller diameter of the said ring (2).

7. Method according to any one of the previous claims, wherein said pressing operations comprise a second moulding operation, in which the edge with smaller diameter of the ring (3) is radially brought into abutment against a centring element (13a), so that the material of the ring (3) is then made to flow radially outwards and longitudinally towards the edge with greater diameter of said ring (3).

8. Method according to one of the previous claims, wherein said pressing operations comprise a moulding operation in which the material of the ring (3) is made to flow radially towards the centre, at the edge with smaller diameter, whereas the material at the edge with greatest diameter is made to flow radially outwards and longitudinally.

9. Method according to any one of the previous claims, wherein said strip of sheet metal (1) is made from steel, in particular steel with low alloying elements content.

10. Method according to claim 11, wherein the strip of sheet metal (1) is made from steel having a manganese content of substantially between 0.15% and 0.80% of the total weight.

## Patentansprüche

1. Verfahren zur Herstellung einer Radscheibe (4) eines Motorfahrzeugs, wobei das Verfahren die folgenden Verfahrensschritt aufweist:
- Bereitstellung eines Metallblechstreifens (1), der im Wesentlichen als ein gestrecktes Parallelogramm mit einer im Wesentlichen gleichmäßigen Dicke geformt ist;
- Biegung des Metallblechstreifens (1) und Verschweißen von dessen Endstücken (1a, 1 b) miteinander, um einen im Wesentlichen zylindrischen Ring auszubilden; und
- Verpressung und Formung des Rings (2) mittels plastischer Deformation, um ihm eine gewünschte Form zu geben; wobei das Verfahren **dadurch gekennzeichnet ist, dass**
- der Metallblechstreifen (1) derartig gebogen wird, dass seine Endstücke (1a, 1b) eben sind;
- die Endstücke (1a, 1b) zusammen gebracht werden und im Wesentlichen in einer gemeinsamen Ebene stumpf verschweißt werden, um einen Ring (2) zu erhalten, der eine abgeflachte Wandung (1a, 1b) aufweist;
- der Ring (2) einem vorläufigen Verrunden unterzogen wird, bevor er der Verpressung und Verformung unterzogen wird,
- das Verrunden durch eine radiale Expansion ausgeführt wird, wobei die Expansion in einem ersten im Wesentlichen zylindrischen axialen Abschnitt (2a) des Rings (2) von einem größeren Ausmaß ist, wobei der übrige axiale Abschnitt (2b) des Ring (2) eine im Wesentlichen kegelförmige Gestalt annimmt.

2. Verfahren nach Anspruch 1, **dadurch gekennzeichnet, dass** der übrige axiale Abschnitt (2b) des Rings (2), der einen im Wesentlichen kegelförmige Gestalt aufweist, eine Erstreckung über circa 25 % der axialen Höhe oder Länge des Rings (2) aufweist.

3. Verfahren nach Anspruch 1 oder 2, **dadurch gekennzeichnet, dass** der Ring (2) nach dem vorläufigen Verrunden und vor der Verpressung und Formung einer Materialentfernung, insbesondere einer Dreharbeit, unterworfen wird, um dessen Höhe oder axiale Länge auf einen vorbestimmten Nennwert zu bringen, und um dessen Endkanten eben und parallel zueinander auszubilden.

4. Verfahren nach Anspruch 3, **dadurch gekennzeichnet, dass** während der Materialentfernung die Ecken der Kanten des Rings (2), die in den nachfolgenden Verfahrensschritten gegen die Form oder Formteile reiben müssen, abgekantet oder abgerundet werden.

5. Verfahren nach einem der vorhergehenden Ansprüche, **dadurch gekennzeichnet, dass** die ebenen Endstücke (1a, 1b) eine derartige Erstreckung haben, dass sie sich in einem Querschnitt jeweils unter einem Winkel (α) zwischen 5° und 15°, und vorzugsweise circa 10°, gegenüberliegen, wobei der Winkel (α) einen Scheitelpunkt auf der Achse (O) des Rings (2) hat.

6. Verfahren nach einem der vorhergehenden Ansprüche, **dadurch gekennzeichnet, dass** die Verpressung einen ersten Verformungsschritt aufweist, der nach dem vorläufigen Verrunden durchgeführt wird, wobei die Kante des Rings (2) mit dem größten Durchmesser axial zur Anlage mit einer Haltefläche (11a) gebracht wird, so dass das Material des Rings (2) gezwungen wird radial in Richtung des Zentrums an der Kante des Rings (2) mit kleinerem Durchmesser zu fließen.

7. Verfahren nach einem der vorhergehenden Ansprüche, **dadurch gekennzeichnet, dass** die Verpressung einen zweiten Verformungsschritt aufweist, in dem die Kante des Rings (3) mit kleinerem Durchmesser radial zur Anlage mit einem Zentrierungselement (13a) gebracht wird, so dass das Material des Rings (2) danach gezwungen wird, radial nach außen und longitudinal in Richtung der Kante des Rings (3) mit größerem Durchmesser zu fließen.

8. Verfahren nach einem der vorhergehenden Ansprüche, **dadurch gekennzeichnet, dass** die Verpressung einen Verformungsschritt aufweist, in dem das Material des Rings (3) gezwungen wird, radial in Richtung des Zentrums an der Kante mit kleinem Durchmesser zu fließen, wohingegen das Material an der Kante mit dem größten Durchmesser gezwungen wird radial nach außen und longitudinal zu fließen.

9. Verfahren nach einem der vorhergehenden Ansprüche, **dadurch gekennzeichnet, dass** der Metallblechstreife (1) aus Stahl, insbesondere aus Stahl mit einem geringen Anteil an Legierungen, ausgebildet ist.

10. Verfahren nach Anspruch 11, **dadurch gekennzeichnet, dass** der Metallblechstreifen (1) aus Stahl gebildet ist, der einen Mangananteil vom im Wesentlichen zwischen 0,15 % und 0,80 % des Gesamtgewichts aufweist.

## Revendications

1. Procédé de fabrication d'un disque (4) pour une roue d'un véhicule à moteur, comprenant les opérations suivantes :
- prendre une bande de tôle (1) substantiellement en forme de parallélogramme allongé ayant une épaisseur essentiellement uniforme ;
- plier ladite bande de tôle (1) et souder entre elles les parties d'extrémité (1a, 1b) de celle-ci afin de former un anneau substantiellement cylindrique ; et
- soumettre ledit anneau (2) à des opérations de pressage et de façonnage par déformation plastique afin de lui donner une forme désirée ;
le procédé étant **caractérisé en ce que** :
- la bande de tôle (1) est courbée de telle manière que ses parties d'extrémité (1a, 1b) sont de niveau ;
- lesdites parties d'extrémité (1a, 1b) sont mises en contact entre elles puis soudées bout à bout substantiellement sur un même plan, afin d'obtenir un anneau (2) qui comporte une partie de paroi aplatie à la corde (1a, 1b) ;
- avant de subir les opérations de pressage et de façonnage susmentionnées, ledit anneau (2) est soumis à une opération d'arrondissage préliminaire,
et **en ce que** :
- ladite opération d'arrondissage est réalisée par expansion radiale de telle sorte que l'expansion est de plus grande amplitude dans une première partie axiale, substantiellement cylindrique, (2a) de l'anneau (2), et la partie axiale restante (2b) de l'anneau (2) prend une configuration substantiellement en forme de cône.

2. Procédé selon la revendication 1, dans lequel la partie axiale restante susmentionnée (2b) de l'anneau (2) qui a une configuration substantiellement en forme de cône s'étend sur environ 25 % de la hauteur ou longueur axiale de l'anneau (2).

3. Procédé selon la revendication 1 ou 2, dans lequel, après l'opération d'arrondissage préliminaire susmentionnée et avant lesdites opérations de pressage et de façonnage, ledit anneau (2) est soumis à une opération de retrait de matière, en particulier une opération de tournage, pour donner à sa hauteur ou longueur axiale une valeur nominale prédéterminée, et pour mettre ses bords d'extrémités de niveau et parallèles entre eux.

4. Procédé selon la revendication 3, dans lequel, dans ladite opération de retrait de matière, les angles des bords de l'anneau (2) qui doivent frotter contre les moules ou formes dans les opérations suivantes sont biseautés ou arrondis.

5. Procédé selon l'une quelconque des revendications précédentes, dans lequel les parties d'extrémités de niveau susmentionnées (1a, 1b) ont une étendue telle que, en section transversale, elles sont sous-tendues chacune par un angle (α) de 5° à 15°, et de préférence d'environ 10°, ledit angle (α) ayant un sommet sur l'axe (0) de l'anneau (2).

6. Procédé selon l'une quelconque des revendications précédentes, dans lequel lesdites opérations de pressage comprennent une première opération de moulage qui est exécutée après ladite opération d'arrondissage préliminaire, et dans laquelle le bord ayant le plus grand diamètre de l'anneau (2) est mis axialement en butée contre une surface d'arrêt (11a), de sorte que l'on fait ensuite s'écouler le matériau de l'anneau (2) radialement vers le centre, au niveau du bord ayant le plus petit diamètre dudit anneau (2).

7. Procédé selon l'une quelconque des revendications précédentes, dans lequel lesdites opérations de pressage comprennent une deuxième opération de moulage, dans laquelle le bord de petit diamètre de l'anneau (3) est mis radialement en butée contre un élément de centrage (13a), de sorte que l'on fait ensuite s'écouler le matériau de l'anneau (3) radialement vers l'extérieur et longitudinalement vers le bord de grand diamètre dudit anneau (3).

8. Procédé selon l'une des revendications précédentes, dans lequel lesdites opérations de pressage comprennent une opération de moulage dans laquelle on fait s'écouler le matériau de l'anneau (3) radialement vers le centre, au niveau du bord de petit diamètre, tandis que l'on fait s'écouler le matériau au niveau du bord de grand diamètre radialement vers l'extérieur et longitudinalement.

9. Procédé selon l'une quelconque des revendications précédentes, dans lequel ladite bande de tôle (1) est en acier, en particulier de l'acier à faible teneur en éléments d'alliage.

10. Procédé selon la revendication 11, dans lequel la bande de tôle (1) est faite d'un acier ayant une teneur en manganèse comprise substantiellement entre 0,15 % et 0,80 % du poids total.
